

April 26, 1938.

J. E. BAUER

2,115,513

WALL CONSTRUCTION

Filed June 23, 1936

FIG-1-



FIG-3-



FIG-2 -



John E. Bauer.  
INVENTOR.

BY *Rule & Hage*  
ATTORNEYS.

## UNITED STATES PATENT OFFICE

2,115,513

## WALL CONSTRUCTION

John E. Bauer, Muncie, Ind., assignor to Owens-  
Illinois Glass Company, a corporation of Ohio

Application June 23, 1936, Serial No. 86,830

9 Claims. (Cl. 72—41)

The present invention relates to improvements in wall construction and is particularly directed towards the provision of a structure possessing an unusually high degree of resistance to excessive pressures of every character.

Wall construction of the type with which the present invention is especially concerned consists of courses of individual blocks which are intended to be bonded together by means of any ordinary good grade of mortar or otherwise.

Outstanding among the objects of my invention is the provision of a bond between the blocks having exceptionally great tensile and shearing strength far exceeding any known or expected in the building trade at the present time.

A further object is the provision of a novel type of mortar bearing surface for building blocks which in addition to greatly facilitating the attainment of an effective bond between the blocks with the use of ordinary good grade mortar, creates a more or less resilient cushion around the mortar bearing surfaces whereby the wall structure is better enabled to withstand wind pressure, expansion and contraction due to temperature changes, and meet the strict specifications of the underwriters for fire testing. Such cushioning additionally functions as a sound deadening medium in that vibrations are not conducted from one block to another in the wall structure to any-thing like the degree ordinarily experienced.

A further object is to provide a coating for the mortar bearing surfaces of sectional building blocks which will have the characteristic of firmly uniting with the bonding medium employed in securing the sections of the block together.

Other objects will be in part apparent and in part pointed out hereinafter.

In the drawing:

Fig. 1 is a fragmentary perspective view of a wall construction built up in accordance with the present invention.

Fig. 2 is a fragmentary detail sectional view showing the joint or bond between the adjacent corners of four blocks.

Fig. 3 is a detail perspective view of one of the blocks.

While the present invention is particularly concerned with wall structure consisting of courses of hollow glass blocks, each comprising sections suitably united and having a reduced internal air pressure, it may with equal facility be adopted in the construction of walls formed from other types of blocks or bricks.

In practicing my invention in accordance with the present disclosure I employ hollow glass

blocks 5 each made up of two rectangular cup-like sections 6, the edge portions 7 of which may be united by a glass-to-glass contact effected while the glass is in a more or less semi-plastic state and quite hot, or by means of a film or sheet 8 of aluminum or some other suitable metal or alloy which is interposed between the edges 7 as a part of the assembly operation. The bottom of each section constitutes a portion of one wall face when the blocks are built up in courses. Because the exterior surface of the blocks is quite smooth, some difficulty would ordinarily be encountered in uniting the blocks in a wall structure which will meet the various requirements of the building codes and withstand necessary pressures, strains and stresses.

I overcome these difficulties by creating an effective mortar bearing surface on those areas ordinarily directly contacted by the mortar. To this end a coating 9 or film of ordinary titanic oxide enamel or some other equivalent oxide, is applied to these areas, after which the block is dipped into sand or some other gritty substance which will provide a rough surface 10 capable of effectively bonding with mortar 11. Obviously, methods other than dipping may be resorted to in applying the gritty substance. Because this particular coating, even after it has dried completely, is yieldable to some extent, it provides a cushion around each block which greatly increases the compressive strength of the wall structure, increases the resistance of the wall to wind pressure and practically insures against cracking or breaking of the wall due to ordinary expansion and construction incident to temperature changes. Further, such a mortar bearing surface, when used in conjunction with an ordinary good grade of mortar in assembling blocks of the above character, has shown the exceptionally high average of 27.2 pounds per square inch in tensile strength (the resistance to separation of the blocks by any relative movement except sliding in the direction of the plane of the surfaces united) as compared with 13.8 pounds per square inch which is required by the ordinary brick code. The shearing strength (the resistance to relative shifting of the blocks in the direction of the plane of the surfaces united) where this particular bond is employed averages approximately 82 pounds per square inch, which is far above any heretofore obtained or at the present time obtainable, with known blocks or bricks and mortar. The compression strength resulting to a considerable extent from the employment of this par-

ticular mortar bearing surface or film, runs as high as two thousand pounds per square inch.

As a base for and in order to materially strengthen the bond between the glass and coating of titanic oxide enamel and grit, I may resort to the application to the mortar bearing surface, of a thin film or coating of metal such for example as aluminum which will effectively adhere to the glass and bonding strip 8 (Fig. 3) 10 which likewise may well be formed of metal such for example as aluminum.

Modifications may be resorted to within the spirit and scope of the appended claims.

I claim:

15 1. A wall structure comprising courses of blocks having glazed surfaces and a bonding medium uniting the blocks and having an average tensile strength of approximately twenty-seven pounds per square inch in the direction of its 20 length and height, said bonding medium including titanic oxide enamel and grit.

2. A wall structure comprising courses of blocks having glazed mortar bearing surfaces, and a bonding medium uniting the blocks and 25 having an average shearing strength in the direction of its thickness of approximately eighty-two pounds per square inch, said bonding medium including grit and an adhesive applied to said surface.

30 3. A wall structure comprising courses of glass blocks and a yieldable bond including titanic oxide enamel and a gritty material uniting the blocks.

4. A wall structure comprising courses of hollow glass blocks, a gritty yieldable coating cover-

ing at least a major portion of the mortar bearing surfaces of the blocks and a mortar uniting the coated areas of adjoining portions.

5 5. A hollow glass building block formed of cup-like sections, a metallic bond uniting the edge portions of the sections, a rough surfaced coating for the mortar bearing surfaces, said coating having characteristics in common with said metallic bond, and a rough surfaced yieldable film overlying and bonded to said coating.

10 6. A building block having normally glazed mortar bearing surfaces and a rough surfaced metallic coating applied to at least a portion of said mortar bearing surface and a rough surfaced yieldable film overlying and bonded to said coating.

15 7. A wall structure comprising courses of blocks having glazed mortar bearing surfaces and means bonding the blocks together including a coating of titanic oxide enamel and grit applied to said surfaces.

20 8. A hollow glass building block formed of sections bonded together and having mortar bearing surfaces bordering the joint between said sections and a coating of adhesive and gritty material over at least a portion of said surfaces.

25 9. A hollow glass building block having mortar bearing surfaces, and a coating bonded to said surfaces and consisting of a film of metal having an affinity for and in part penetrating the glass, 30 an oxide enamel adhering to the metal and a gritty material dispersed over and adhering to said enamel and providing a rough exposed surface.

JOHN E. BAUER. 35